

## UNITED STATES PATENT OFFICE

1,986,767

## STEEL AND METHOD OF MAKING THE SAME

Wilbert F. Davis and George E. Hitchens, McKeesport, Pa., assignors to National Tube Company, a corporation of New Jersey

No Drawing. Application March 21, 1933,  
Serial No. 662,000

6 Claims. (Cl. 75—45)

This invention relates to an improved steel and method of making the same.

One object of the present invention is to provide a steel having desirable characteristics heretofore unobtainable by any of the well known methods. It is a well known fact that "open-hearth steel" and "Bessemer steel" are each possessed of certain desirable characteristics not found in the other; as, for instance, the former is more ductile than the latter.

In the manufacture of certain classes of tubular products, such as conduit, etc., it is found that Bessemer steel will thread and electroplate very satisfactorily, but is stiff and brittle and consequently hard to bend. Open-hearth steel, on the other hand, will bend more easily but does not thread or electroplate as satisfactorily as Bessemer steel. Accordingly, it has been the practice in the past to select the steel having the most desirable characteristics for certain purposes, which has meant, of course, that, while not quite so marked, certain undesirable features must necessarily be present. In accordance with the teachings of the present invention, however, these difficulties are obviated and a steel is obtained having all of the desirable characteristics.

Another object is to provide a method of making steel in which the physical properties of the metal may be more satisfactorily controlled, particularly the phosphorus content, which has an effect upon ductility and consequently produces a steel which will bend easily without being brittle.

35 The improved steel of the invention is characterized by including the following elements in substantially the proportions specified:

|                     |            |
|---------------------|------------|
| Carbon              | .04 to .09 |
| Manganese           | .30 to .60 |
| Phosphorus not over | .060       |
| Sulphur not over    | .060       |

40 and may be obtained in a number of different ways as, for example, by adding phosphorus, sulphur and manganese to a low carbon steel.

45 However, the steel of the invention may be obtained by mixing low carbon basic open hearth steel and low carbon acid Bessemer steel. The method of obtaining the two steels to be mixed is done in accordance with conventional practice, and as such forms no part of the present invention.

For the purposes of illustration, an analysis of a typical heat of each of the two steels is as follows:

## Low carbon basic open-hearth steel

|            |      |
|------------|------|
| Carbon     | .03  |
| Manganese  | .11  |
| Phosphorus | .005 |
| Sulphur    | .031 |

5

## Low carbon acid Bessemer steel

|            |      |
|------------|------|
| Carbon     | .03  |
| Manganese  | .07  |
| Phosphorus | .069 |
| Sulphur    | .035 |

10

The two steels are mixed together in a ladle by adding the Bessemer steel to the open-hearth steel, or adding the open-hearth steel to the Bessemer steel, but preferably by pouring the Bessemer steel into the open-hearth steel, as this retains the gases which are present in the former and allows them to escape after being "teemed" from the ladle into a mold, which causes the proper rimming action and solidification of the ingot.

Immediately the open-hearth steel is poured into the ladle, any portion of the required ferro-manganese is added. The ladle is then transferred to the Bessemer converter, which has been blown in the usual manner. The Bessemer steel is then poured into the ladle containing the open-hearth steel and the remaining portion, if any, of the ferro-manganese is added. The steel mixture may then be "teemed" from the ladle into suitable molds.

An analysis of the mixture of the above referred to typical heats of open-hearth and Bessemer steels is as follows:

## Mixed steel

|            |      |
|------------|------|
| Carbon     | .07  |
| Manganese  | .35  |
| Phosphorus | .039 |
| Sulphur    | .032 |

40

The change in the analysis of carbon and manganese in the mixed steel is due to the carbon and manganese in the ferro-manganese which is added to the ladle. This gives the desired carbon and manganese in the finished steel.

It is to be understood that by varying the proportions of each steel that the phosphorus content may be changed, and by recarburizing with ferro-manganese or other recarburizers in the ladle a steel can be produced with varying amounts of manganese and carbon. The sulphur and silicon is practically the same in both

50

45

55

the open-hearth and Bessemer steels, and remains the same in the mixed steel. These ingredients can also be varied by adding sulphur or ferro-silicon to the ladle.

5 In the manufacture of tubular products the physical properties of the metal are tested by subjecting the crop-ends of the product to crushing between parallel plates to one-third of its diameter. If the product cracks at the point 10 of maximum bend it is rejected. A comparison of acceptable ductility between the results of crushing tests on the various steels is as follows:

|                               |        |
|-------------------------------|--------|
| Open-hearth steel             | 100.00 |
| Bessemer steel                | 75.7   |
| 15 The steel of the invention | 97.3   |

Experience has shown that when the steel of this invention is made by mixing low carbon basic open-hearth steel and low carbon acid 20 Bessemer steel in the ladle the Bessemer steel must be poured into the open-hearth steel in order to secure the desired results. When the Bessemer steel is poured into the open-hearth steel the gases present in the Bessemer steel are retained and allowed to escape only after 25 being "teemed", which causes the proper "rimming" action and solidification of the ingot. The steel resulting from this method of mixing when subjected to crushing tests proves to be 30 substantially as ductile as open-hearth steel or, in other words, 97.3, as compared with open-hearth steel at 100. If the order of mixing is reversed, and low carbon basic open-hearth steel is poured into low carbon acid Bessemer 35 steel, the ductility of the resulting steel would prove to be only 57.1 when compared with open-hearth steel.

This latter result is due to the fact that when the basic open-hearth steel is poured into the acid Bessemer steel the gases in the Bessemer steel are partly removed by the violent agitation 40 of the metal, and there is not sufficient action when teemed into the mold to allow the gases to escape, consequently making a tendency for 45 the steel to rise in the mold, which causes the blow holes to be too close to the surface. This, of course, results in a product with a defective surface, and one which does not have the required physical properties.

50 While we have shown and described several specific embodiments of our invention it will be understood that we do not wish to be limited exactly thereto, since various modifications may be made without departing from the scope of our invention, as defined in the following claims.

55 We claim:

1. The method of making steel containing

approximately .04 percent to .09 percent carbon; .30 to .60 percent manganese; less than .060 percent phosphorus; less than .060 percent sulfur; the remainder being iron and the usual traces of residual ingredients such as silicon which includes adding low carbon Bessemer steel to a substantially equal quantity of low carbon basic open-hearth steel. 5

2. The method of making steel containing approximately .04 percent to .09 percent carbon; .30 to .60 percent manganese; less than .060 percent phosphorus; less than .060 percent sulfur; the remainder being iron and the usual traces of residual ingredients such as silicon which includes recarburizing low carbon open-hearth 10 steel, and adding thereto a substantially equal quantity of low carbon Bessemer steel. 15

3. The method of making steel containing approximately .04 percent to .09 percent carbon; .30 to .60 percent manganese; less than .060 percent phosphorus; less than .060 percent sulfur; the remainder being iron and the usual traces of residual ingredients such as silicon which includes recarburizing low carbon open-hearth 20 steel, adding thereto a substantially equal quantity of low carbon Bessemer steel, and recarburizing the combined open-hearth and Bessemer steels. 25

4. The method of making steel containing approximately .07 percent carbon; .35 percent manganese; .039 percent phosphorus; .032 percent sulfur, the remainder being iron and the usual traces of residual ingredients, such as silicon, which includes adding low carbon Bessemer steel to a substantially equal quantity 35 of low carbon basic open-hearth steel.

5. The method of making steel containing approximately .07 percent carbon; .35 percent manganese; .039 percent phosphorus; .032 percent sulfur; the remainder being iron and the usual 40 traces of residual ingredients such as silicon, which includes recarburizing low carbon open-hearth steel, and adding thereto a substantially equal quantity of low carbon Bessemer steel.

6. The method of making steel containing 45 approximately .07 percent carbon; .35 percent manganese; .039 percent phosphorus; .032 percent sulfur; the remainder being iron and the usual traces of residual ingredients such as silicon, which includes recarburizing low carbon 50 open-hearth steel, adding thereto a substantially equal quantity of low carbon Bessemer steel, and recarburizing the combined open-hearth and Bessemer steels.

WILBERT F. DAVIS.  
GEORGE E. HITCHENS.

55